

## UNITED STATES PATENT OFFICE

2,000,603

TREATMENT OF CELLULOUS MATERIAL  
PRIOR TO ESTERIFICATIONCarl J. Malm and Charles R. Fordyce, Rochester,  
N. Y., assignors to Eastman Kodak Company,  
Rochester, N. Y., a corporation of New YorkNo Drawing. Application February 18, 1932,  
Serial No. 593,870

12 Claims. (Cl. 260—101)

The present invention relates to the preparation of cellulosic material for esterification by treating it with liquid sulfur dioxide with or without a catalyst such as sulfuric acid.

5 The usual processes of esterifying cellulosic material may be divided into the two classes of the dope-forming and the non-dope-forming or fibrous processes. In the fibrous processes when carried out in a liquid bath it is essential that 10 a sufficient amount of a non-solvent be added to render the bath non-solvent of the cellulose ester which is to be prepared. Heretofore the cellulosic material employed as the starting material for esterification has been as a rule pretreated with a bath comprising substantially 15 glucal acetic acid. Glacial acetic acid is a solvent for practically all of the organic esters of cellulose so that in the case of fibrous esterification processes sufficient non-solvent is necessary 20 to overcome the solvent effects of the acetic acid. The removal of acetic acid, more than that which can be pressed off from the cellulose, is commercially impractical as is well known to 25 those skilled in the art.

It has been previously known to pretreat cellulose with  $\text{SO}_2$  in a bath substantially comprising glacial acetic acid and containing only a small amount of  $\text{SO}_2$  gas dissolved therein, with 30 or without a catalyst. However that process has the same disadvantages as far as the fibrous esterification of cellulose is concerned as the pretreatment processes of the prior art in which no  $\text{SO}_2$  is employed. In addition the  $\text{SO}_2$  in that 35 process is present as an impurity in the acetic acid necessitating its removal in the reclamation of the acetic acid employed.

One subject of our invention is to reduce the 40 manufacturing costs of cellulose acetate when prepared by fibrous esterification processes. Another object of our invention is to provide a process in which the esterification of the cellulose is accomplished within a moderate space 45 of time and which results in a uniformly excellent product. Another object of our invention is to provide a process for the pretreatment of cellulose prior to its esterification which need not contribute any re-agents to the esterification 50 bath proper thus making possible the employment of the particular esterification desired, whether by vapor or liquid bath, fibrous or dope-forming and in which the solvents, anhydrides, diluents, catalysts etc. desired may be employed 55 depending merely on the judgment and skill of

the individual operator. Various other objects will appear hereinafter.

We have found that cellulose can be made more readily reactive by treating it with a bath 5 substantially comprising liquid  $\text{SO}_2$  with or without a catalyst. We have found that cellulose may be prepared for esterification without the use of glacial acetic acid in the pretreatment bath. We have found that by our 10 invention all or substantially all of the pretreating liquid may be removed from the cellulose prior to its esterification so that the character 15 of the esterification bath is affected little if at all by the liquid bath employed for the pretreatment. We have found that by our invention the same pretreating liquid may be easily 20 recovered and employed for treating each successive batch of cellulose which it is desired to 25 esterify.

We have found that our pretreatment process 30 is especially valuable where a fibrous esterification is contemplated in which as little non-solvent as possible is desired. As  $\text{SO}_2$  is a gas at ordinary temperature it may be substantially all removed from the cellulose which has been 35 pretreated before the addition of the esterifying bath comprising the non-solvent and the anhydride so that the amount of nonsolvent necessary is considerably less than is the case 40 of the fibrous esterification of a cellulose which has been pretreated in the usual manner.

The pretreatment of cellulose according to 45 our invention is carried out preferably in a closed vessel and when temperatures above the boiling point of the  $\text{SO}_2$  are used, in a pressure vessel. If a catalyst, such as sulfuric acid, is present in the bath the cellulose may be treated at a temperature below the boiling point of the  $\text{SO}_2$  at atmospheric pressure. However when the pretreatment is carried out without the catalyst it is preferred that a higher temperature be employed in order to shorten the time of treatment. In such case it would be desirable to carry out the pretreatment in an enclosed pressure vessel to avoid breakage or the loss of  $\text{SO}_2$ . Obviously the pressure would then be above atmospheric. If desired the pretreatment could however be carried out in a refluxing apparatus in which case the condensing portion 50 must necessarily be at a rather low temperature such as may be obtained by the circulation of a brine having a temperature of  $0^{\circ}$  F. At the end of the pretreatment the  $\text{SO}_2$  may be removed 55 from the cellulose by distillation which due to

the low boiling point of the SO<sub>2</sub> is a relatively simple matter.

It is not known whether sulfur dioxide has the same effect on cellulose in the pretreatment as does acetic acid or not but the pretreated cellulose is readily esterified and gives cellulose esters of extraordinary whiteness. The fact that liquid SO<sub>2</sub> may be employed in the pretreatment of cellulose is remarkable when it is considered that sulfur dioxide bears no relation chemically to glacial acetic acid which has been usually employed heretofore.

One feature of our invention which is of importance from the economic standpoint is that the SO<sub>2</sub> which is employed in the pretreatment of cellulose may be recovered in a pure form in practically its entirety, from the pre-treated cellulose and thus the same SO<sub>2</sub> may be employed over and over again for pretreating successive batches of cellulose. If a catalyst such as sulfuric acid is incorporated with the SO<sub>2</sub> in the pretreatment bath, upon distillation off of the SO<sub>2</sub> this foreign material remains on the cellulose where it may act as a catalyst in the subsequent esterification. Thus only the pure SO<sub>2</sub> distills off from the cellulose.

As has been pointed out above, our pretreatment may be employed to prepare cellulose for either dope-forming or fibrous esterification processes, and the esterification bath may be of any composition disclosed in the prior art. For example our pretreated cellulose may be employed for either the preparation of cellulose acetate by the use of acetic anhydrid or acetyl chlorid or it may be employed as the starting material for the preparation of higher esters (either simple or mixed) for instance according to one of the processes disclosed in U. S. Patents Nos. 1,800,860 and 1,880,808 of Clarke & Malm.

The following example illustrates the application of our pretreatment to a process for the fibrous esterification of cellulose:

50 lbs. of cotton linters was mixed with 290 lbs. of liquid SO<sub>2</sub> containing 2 lbs. of sulfuric acid and the whole was maintained at a temperature of 10° F. for 10 hours. The excess SO<sub>2</sub> was drained off and the temperature was then allowed to rise until the SO<sub>2</sub> remaining was distilled off. This SO<sub>2</sub> was condensed and employed in a subsequent pretreatment.

The pretreated cellulose was then added to a mixture of 150 lbs. of acetic anhydrid and 630 lbs. of carbon tetrachlorid and the mass was maintained at a maximum temperature of 40° C. until a sample showed that the ester formed was soluble in a mixture consisting of chloroform-ethyl alcohol containing 15% of the latter.

60 The use of carbon tetrachlorid as the non-solvent in the example is merely illustrative as any of the known non-solvents such as benzene or a higher ether as disclosed in Malm and Fletcher application Serial No. 590,508, filed February 2, 1932 may be employed.

70 The cellulose which is employed as the starting material may be any of the usual types disclosed in the prior art such as pulp, linters or other forms. This starting cellulose is preferably one which has been bleached and oven-dried and which contains not more than about 1% of moisture.

75 Various other modifications of our invention which are apparent to those skilled in the art such as the use of different catalysts, variations

in proportions, time of treatment, etc. are within the scope of the present invention. For example the liquid SO<sub>2</sub> might be mixed with non-solvent such as carbon tetrachlorid, a higher ether or the like and the pretreatment of the cellulose would take place in that bath with or without a catalyst. After the pretreatment the SO<sub>2</sub> may be easily removed from the carbon tetrachloride by allowing the mixture to come to room temperature. The SO<sub>2</sub> distills off and can be collected for reuse. The cellulose remaining is wet with carbon tetrachlorid (or the other non-solvent employed) and is eminently fitted for use as the starting material in a fibrous esterification bath.

15 If desired the carbon tetrachlorid could also be removed from the cellulose after this type of pretreatment by mild heating at a temperature above the boiling point of the tetrachlorid and below that point at which the cellulose is scorched or affected detrimentally. This cellulose from which the pretreating liquid is removed may then be employed in dope esterification processes.

20 Obviously if desired a small amount of glacial acetic acid might also be dissolved in the liquid SO<sub>2</sub> to form a pretreatment bath, from which at the end of the pretreatment the SO<sub>2</sub> could be all removed. This type of pretreatment bath is adapted for the preliminary treatment of cellulose for dope esterification processes as the pre-treated cellulose in this case has a certain content of glacial acetic acid homogeneously distributed therethru.

25 We claim as our invention:

30 1. The preparation of cellulose for esterification which comprises pretreating it with a bath containing liquid sulfur dioxide as the principal active pretreating agent preliminary to the application of esterifying reagents thereto.

35 2. The preparation of cellulose for esterification which comprises pretreating it with a bath containing a predominating proportion of liquid sulfur dioxide preliminary to the application of esterifying reagents thereto.

40 3. The preparation of cellulose for esterification which comprises pretreating it with a bath containing a predominating proportion of liquid sulfur dioxide and a small amount of catalyst preliminary to the application of esterifying 45 reagents thereto.

45 4. The preparation of cellulose for esterification which comprises pre-treating it with a bath containing a predominating proportion of liquid sulfur dioxide and a small amount of sulfuric acid preliminary to the application of esterifying 50 reagents thereto.

55 5. The preparation of cellulose for esterification which comprises pretreating it with a bath containing a predominating proportion of liquid sulfur dioxide and a small amount of sulfuric acid at a temperature below the boiling point of the sulfur dioxide preliminary to the application of esterifying reagents thereto.

60 6. In the esterification of cellulose the steps which comprises pretreating the cellulose with a bath containing a predominating proportion of liquid sulfur dioxide under conditions whereby the sulfur dioxide retains its liquid state and then restoring normal conditions so that the SO<sub>2</sub> 65 may evaporate off from the cellulose.

70 7. A process for the fibrous esterification of cellulose which comprises treating the cellulose with a bath comprising mainly liquid sulfur dioxide, removing the sulfur dioxid and then 75

esterifying the cellulose in a bath substantially comprising a fatty acid anhydrid, a non-solvent and a catalyst.

8. A process for the fibrous acetylation of cellulose which comprises treating the cellulose with a liquid sulfur dioxide bath, removing the sulfur dioxide and then esterifying the cellulose in a bath substantially comprising acetic anhydrid, a non-solvent and a catalyst.

10. 9. In the preparation of cellulosic materials for esterification the cyclic process of treating the cellulosic material with liquid sulfur dioxide, then draining off some of the liquid sulfur dioxide from the cellulose and distilling off the

15 remainder, and treating a second batch of cellulosic material with a bath substantially comprising the recovered sulfur dioxide in liquid form.

10. The preparation of cellulose for esterification which comprises pretreating it with a bath containing a predominating proportion of liquid sulfur dioxide at a pressure above atmospheric.

11. In the process of making cellulose acetate, the step which comprises pretreating the cellulose to be acetylated with a preliminary bath containing a predominating proportion of liquid sulfur dioxide.

12. A process for the fibrous esterification of cellulose which comprises treating the cellulose with a bath comprising mainly liquid sulfur dioxide, removing the sulfur dioxide and then esterifying the cellulose.

10

15

CARL J. MALM.  
CHARLES R. FORDYCE.